

## UNITED STATES PATENT OFFICE

2,049,217

PROCESSES OF IMPREGNATING  
CELLULOSIC FABRICS

Pierre Meunier, Paris, France, assignor to Resines et Vernis Artificiels (Societe Anonyme), Lyon, Rhone, France, a company of France

No Drawing. Application March 27, 1934, Serial No. 717,681. In France March 31, 1933

6 Claims. (Cl. 91—70)

It has been known for a long time that various properties of fabrics of any kind and more especially cellulosic fabrics could be improved by impregnating them with synthetic resins that are soluble and subsequently polymerizing these resins through the action of heat.

The first applications of this method were made with resins obtained by condensation of phenols with formaldehyde, by utilizing the so-called bakelization process.

The most important patent that was taken for protecting a method of this kind is the German Patent No. 318,509 to Gunther, filed June 20, 1914. This method describes a method of dressing fabrics by impregnating them with the condensation products of phenols and formaldehyde that are soluble in water (for instance equal weights of phenol and formaldehyde of 40%, condensed in the presence of an alkali and having a total concentration in resin of 30%).

The same principle was applied by Ruff to the treatment of paper fabrics (German Patents No. 302,551 of July 6, 1917, No. 303,926 of March 21, 1917, No. 327,399 of October 27, 1917). More recently, the Tootal Broadhurst Company (British Patents No. 291,473, 291,474 and 304,900) improved the method of Gunther by performing a preliminary mercerizing of the fabric, and treating the product in a boiling soap bath after polymerization in order to facilitate, on the one hand, the penetration of the resin in the fibre and, on the other hand, the elimination of the excess of phenol and of the soluble condensation products.

Other methods, including the impregnation of fabrics of any kind whatever with phenolic synthetic resins have been proposed by Blumer (German Patent No. 174,745) and Bucherer (German Patent No. 339,301 of August 24, 1918).

By treating cotton and artificial silk fabrics according to the method set forth in the German Patent No. 318,509 to Gunther, the stiffening produced on the fabric permits the easy fixation of the colouring materials and this stiffening is permanent, that is to say is not destroyed by washing and resists rumpling.

However, the utilization of formaldehyde and phenol resins permits the application of the method only in the case of dark shades because of the oxidation of the traces of phenol that are not combined under the influence of light, and of the alteration of the colors that results therefrom.

When synthetic resins other than phenol formaldehyde condensation products were discovered, it was endeavoured to apply them to the

impregnation of fabrics with a view to obtaining permanent stiffening compounds having more or less interesting practical properties.

In the German Patent No. 556,393, filed in the name of the Cotton Treating Syndicate, which patent corresponds to the British Patent No. 258,357, filed June 19, 1925, fabrics are impregnated with the soluble condensation products of thio-urea and formaldehyde, in the presence of filling materials, and polymerization takes place subsequently under the action of heat in the presence of an acid agent.

This process, the principle of which is substantially the same as that of Gunther for phenolic resins, is chiefly intended to fix the filling materials on the fabrics but it produces, as the Gunther process, a permanent stiffening matter which resists washing and rumpling. However, this process has the disadvantage of being somewhat expensive, due to the utilization of thio-urea.

I may also cite the German Patents No. 535,234 of October 6, 1926, and No. 537,036 of July 26, 1927, filed by the I. G. Farbenindustrie, concerning the treatment of freshly precipitated hydro-cellulose. Drying is effected by means of solutions of dimethylol-urea with a view to reducing the power of swelling of the threads of artificial silk.

The British Patent No. 291,473, of December 1, 1926, teaches impregnating fabrics with soluble resins resulting from the condensation of ordinary urea with formaldehyde. The general process is very much the same as that disclosed by the Patents No. 318,509 (Gunther) and No. 556,393 (Cotton Treating Syndicate); however it includes a preliminary mercerizing in order to facilitate the penetration of the resin.

Fabrics treated according to the processes above mentioned have more or less different qualities according to the nature of the resins that are utilized, the concentration of the resin solutions, etc., but they are permanently stiffened or dressed, that is to say they are capable of resisting washing and rumpling.

For practical purposes use will be made of resins giving, to the maximum degree, the permanency of the stiffening (that is to say the resistance to washing and rumpling), and the properties of plasticity of the resins that are employed will play an important part.

One shall thus preferably utilize resins capable of preserving the original aspect and feel of the fabrics, as far as possible, and which will have

a great stability in the state of solutions, in order to facilitate their use.

The present invention concerns a process of impregnating fabrics with a particularly advantageous kind of resins with a view to obtaining a permanent stiffening capable of resisting rumpling while preserving the flexibility of the fabric and a good feel thereof. The resins that are utilized according to the present invention have the further advantage that they necessitate no preliminary treatment of the fabrics (even in the case of cotton fabrics), said fabrics being merely impregnated with the resin that is used and then subjected to a polymerizing treatment by means of heat, in a manner similar to that taught by Gunther, either in the presence of a catalyst or not. They further possess the advantage of having a good stability when in solution.

The resins that are employed for the treatment of fabrics according to the present invention are obtained by condensation of formaldehyde with ammonium sulphides or ammonium sulphocyanide, in the presence of variable quantities of urea, or by condensation of thioaldehydes with urea.

As a matter of fact, ammonium sulphide can combine with formaldehyde without disengagement of sulphuretted hydrogen so as to give compounds of the type of sulphines (pentamethylene-diamine-disulphine and thiadines, Delépine, A. Ch. vol. 15, p. 570-574 and thesis 1898, p. 101). If the condensation of these bodies is furthered by heat, resinous products having a great elasticity are obtained.

When this condensation takes place in the presence of variable quantities of urea, resins are obtained which differ from resins resulting from the condensation of urea or thiourea with formaldehyde by their chemical composition and their properties.

In particular they are neither gelatinized nor precipitated in concentrated solution by the addition of sulphuric acid of 50% or by heating in the presence of ammonium sulphocyanide, while, in the case of urea-formaldehyde, or thio-urea-formaldehyde resins, an instantaneous precipitation takes place.

For carrying out the process according to the present invention, the resins above referred to are prepared in the state of aqueous solutions only little condensed (for instance by causing the reagents to act on one another in the cold state) and diluted in such manner as to obtain a suitable concentration, which varies with the nature of the fabrics to be treated and of the final effect to be obtained. This concentration may range between 10 and 30 per cent. Colouring materials, fillers, plastifiers or softening matters may be eventually added to the solutions, and the fabric is immersed into the bath while suitably stirring it.

It should be noted that interesting results are obtained by making use of the products of the simple condensation of formaldehyde with ammonium sulphides or ammonium sulphocyanide, for instance by impregnating a fabric of viscose silk, or copper silk, with a solution containing 100 parts of formaldehyde of 30%, 50 parts of ammonium sulphocyanide and 50 parts of water and by heating in a closed vessel at a temperature of 80° C. for an hour the fabric freed from the excess of liquid, and then completing polymerization through the action of heat or by immersing the fabric in a bath of formaldehyde containing 40%

in volumes of formaldehyde, removing the excess of liquid from the fabric, dipping in a bath of ammonium sulphide of 30% containing 10% of ammonium sulphocyanide, then removing the excess of liquid from the fabric, drying and polymerizing through the action of heat.

However the best results for practical purposes are obtained with resins resulting from the condensation of formaldehyde with ammonium sulphides or ammonium sulphocyanide in the presence of urea, some properties of which condensation products have been stated above.

In any case, the final polymerization of the resin with which the fabric has been treated is performed through the action of heat at a temperature which may range between 70 and 160° C., for instance by causing the fabric to pass over heated cylinders.

In the processes above cited, which make use of condensation products of urea, it is necessary, in order to obtain polymerization, to treat either for half an hour at a temperature of 130° or for several minutes at a temperature of 160-180° C.

Now, if the polymerizing treatment is to last for half an hour it is very difficult to work in a continuous fashion and if this treatment is to take place at temperatures ranging between 160 and 180° C., the properties of the fabric are very much altered.

On the contrary, according to the present invention, the same degree of polymerization is obtained by a treatment of say one minute at a temperature of 120° C.

*Example I.*—A viscose fabric is impregnated in a solution containing 900 parts in weight of formaldehyde of 30%, 300 parts of urea, 150 parts of ammonium sulphide of 30%, 70 parts of ammonium sulphocyanide and 900 parts of water. The fabric is freed from the excess of water, then dried and the resin with which it is impregnated is polymerized by causing the fabric to pass over rollers heated at a temperature of 130° C. The fabric thus obtained has a very good feel and resists rumpling.

*Example II.*—A fabric is impregnated with a solution containing 500 parts of formaldehyde of 30% in weight, 150 parts of urea, 300 parts of ammonium sulphide of 30% and 2000 parts of water. The fabric is freed from the excess of water and then dried for ten minutes at a temperature of 150° C.

*Example III.*—A viscose fabric is impregnated in a solution containing 900 parts of formaldehyde of 30%, 300 parts of urea, 150 parts of ammonium sulphide of 30%, 1000 parts of water, 60 parts of sulphonated cetyl alcohol, 50 parts of ammonium sulphocyanide, and 20 parts of pure azol blue. The fabric is then treated as in Example II.

*Example IV.*—The fabric is impregnated as in Examples I and II, then freed from the excess of water and dried. It is then caused to pass over smooth cylinders heated at a temperature of 100° C. Finally polymerization of the resin is completed by causing the fabric to pass on engraved cylinders heated at a temperature of 150° C. The dressed and goffered fabric thus obtained is capable of resisting flattening and rumpling actions.

What I claim is:

1. The process of treating woven or knitted cellulosic textile fabrics to enable them to resist creasing and rumpling while retaining their flexibility, which comprises the steps of impreg-

nating such fabric in aqueous solution in the cold state, with a soluble condensation product resulting from the reaction of formaldehyde with a sulphur containing ammonium salt of the 5 group consisting of ammonium sulphides and ammonium sulphocyanide, and then polymerizing the condensation product impregnated in the fabric by heating the impregnated fabric to a temperature of between 70° and 160° C.

- 10 2. The process of treating woven or knitted cellulosic textile fabrics to enable them to resist creasing and rumpling while retaining their flexibility, which comprises the steps of impregnating such fabric in aqueous solution in the cold 15 state, with a soluble condensation product resulting from the reaction of formaldehyde with a sulphur containing ammonium salt of the group consisting of ammonium sulphides and ammonium sulphocyanide in the presence of urea, and then polymerizing the condensation product impregnated in the fabric by heating the impregnated fabric to a temperature of between 100° C. to 150° C. for a period of not over ten minutes.

- 20 3. The process of treating woven or knitted cellulosic textile fabrics to enable them to resist creasing and rumpling while retaining their flexibility, which comprises the steps of impregnating such fabric in aqueous solution in the cold 25 state, with a soluble condensation product resulting from the reaction of formaldehyde with ammonium sulphide, and then polymerizing the condensation product impregnated in the fabric by heating the impregnated fabric to a temperature of between 100° C. to 150° C. for a period 30 of not over ten minutes.

- 35 4. The process of treating woven or knitted cellulosic textile fabrics to enable them to resist creasing and rumpling while retaining their flexibility, which comprises the steps of impregnating such fabric in aqueous solution in the cold 40 state, with a soluble condensation product re-

sulting from the reaction of formaldehyde with ammonium sulphocyanide, and then polymerizing the condensation product impregnated in the fabric by heating the impregnated fabric to a temperature of between 100° C. to 150° C. for a 5 period of not over ten minutes.

5. The continuous process of treating woven or knitted cellulosic textile fabrics to enable them to resist creasing and rumpling while retaining their flexibility, which comprises passing the fabric in the cold state through a bath which consists of a substantially neutral aqueous solution of a soluble condensation product resulting from the reaction of formaldehyde with a sulphur containing ammonium salt of the group consisting of ammonium sulphides and ammonium sulphocyanide in the presence of urea, removing excess liquid from the fabric, drying it, and polymerizing the condensation product impregnated in the fabric by continuously subjecting successive portions of the impregnated fabric to a temperature of from approximately 120° C. to 150° C. for from approximately 1 to 2 minutes.

6. The continuous process of treating woven or knitted cellulosic textile fabrics to enable them to resist creasing and rumpling while retaining their flexibility, which comprises passing the fabric in the cold state through a bath which consists of a substantially neutral aqueous solution of a soluble condensation product resulting from the reaction of formaldehyde with a sulphur containing ammonium salt of the group consisting of ammonium sulphides and ammonium sulphocyanide in the presence of urea, removing excess liquid from the fabric, drying it, continuously passing the fabric over smooth cylinders heated to approximately 100° C. and then completing the polymerization by passing the cloth over cylinders heated to approximately 150° C.

PIERRE MEUNIER.